

# UNITED STATES PATENT OFFICE.

WIKTOR VON FLORYANOWICZ, OF WARSAW, RUSSIA.

## PROCESS OF PRODUCING ARTIFICIAL EMERY.

SPECIFICATION forming part of Letters Patent No. 601,246, dated March 29, 1898.

Application filed April 12, 1897. Serial No. 631,846. (No specimens.)

*To all whom it may concern:*

Be it known that I, WIKTOR VON FLORYANOWICZ, a subject of the Emperor of Russia, residing at Warsaw, Russia, have invented 5 certain new and useful Improvements in Processes of Producing Artificial Emery, of which the following is a specification.

This invention refers to the manufacture of artificial grinding and polishing material 10 and in grinding-wheels, grindstones, and other tools made therewith. This material forms an excellent substitute for emery and is applicable to the grinding and polishing of very hard substances, such as porcelain, glass, and 15 steel.

For producing the material I intimately mix purified fire-clay with water, so as to form a pasty mass, which I dry and then burn at a temperature of about 1,200° to 1,300° centigrade. (1,200° centigrade equals 2,192° Fahrenheit and 1,300° centigrade equals 2,372° Fahrenheit.) The result is a uniformly hard product having a hardness of eight to nine 20 on the Mohrs scale, or equal to that of emery. If it should happen in case of fire-clay of various qualities that it does not melt at 1,200° to 1,300° centigrade, then I add about ten per 25 cent. of feldspar or two per cent. burnt lime. The burnt clay is ground by rolls or edge-runners and sieved through various fine sieves, so that powders of different fineness are obtained, which are equal in hardness to the Naxos emery and can be similarly applied.

To make grinding or polishing wheels or 30 grindstones from this material, I mix intimately forty per cent. of the grinding-powder with forty-five per cent. of ground fire-clay and fifteen per cent. of manganese and moisten the mixture with water, press into shape 35 in molds, dry the objects so made, and burn them at a heat of about 800° centigrade. (800° centigrade equals 1,472° Fahrenheit.) The addition of manganese serves to give the 40 wheels or grindstones a darker color.

The material made by the process described 45 is half the cost of Naxos emery, grinds hard materials better than the said emery, and is more durable. It has also the advantage

that hardened steel treated therewith does not lose its hardness and that but little dust is 50 made.

This new material may be glued onto canvas, leather, or paper.

Having now particularly described and ascertained the nature of my said invention and 55 in what manner the same is to be performed, I declare that what I claim is—

1. The process herein described of manufacturing a grinding and polishing material 60 adapted for making grindstones, grinding-wheels and the like, the said process consisting in burning purified fire-clay, mixed with a small percentage of feldspar or burnt lime, at a temperature of about 1,200° to 1,300° centigrade and then grinding the burned material to reduce it to the desired condition of 65 fineness.

2. The process herein described of manufacturing grindstones and other grinding-tools, said process consisting in burning purified fire-clay at a temperature of about 1,200° to 1,300° centigrade, grinding the burned material, mixing the same with fire-clay and water to form a paste, pressing the same in molds, and burning the objects molded at a 75 temperature of about 800° centigrade, substantially as set forth.

3. The process herein described of manufacturing grindstones and other grinding-tools, said process consisting in mixing with 80 purified fire-clay a small percentage of feldspar or burnt lime, burning the mixture at a temperature of about 1,200° to 1,300° centigrade, grinding the burned material, mixing the same with fire-clay and water to form a 85 paste, pressing the same in molds, and burning the objects molded at a temperature of about 800° centigrade, substantially as set forth.

In testimony whereof I have signed my 90 name to this specification in the presence of two subscribing witnesses.

WIKTOR V. FLORYANOWICZ.

Witnesses:

W. HAUPT,  
HENRY HASPER.